

# United States Patent Office

3,005,736

Patented Oct. 24, 1961

1

3,005,736

## HIGH-TOUGHNESS CAST-IRON FOR RELATIVELY THICK CASTINGS, AND METHOD OF PRODUCING SAME

Lucien Pera, Billancourt, France, assignor to Regie Nationale des Usines Renault, Billancourt, Seine, France  
No Drawing. Filed Jan. 30, 1959, Ser. No. 790,038  
Claims priority, application France Feb. 6, 1958  
1 Claim. (Cl. 148—35)

In prior patent applications, such as those which have issued as U.S. Patents Nos. 2,895,860 and 2,899,346, I have described a method of producing ferrous metal castings having novel and improved properties, wherein the graphite is diffused in the form of a large number of small particles, the mechanical properties of the metal thus obtained being such that in many cases the cast-iron of this specific quality may be substituted for steel. These results are due essentially to the application of a special thermal treatment comprising the following successive steps: austenitization, martensitic hardening, germination heating at a critical effect temperature, followed by graphitization heating at a temperature above the temperature of eutectoid transformation.

This method is particularly suitable for the manufacture of thin castings, for example of a thickness of  $\frac{3}{4}$ " or less.

Now it is the object of this invention to provide specific means whereby the advantageous results obtained with the method broadly set forth hereinabove may be reproduced in the fabrication of massive or relatively thick castings such as internal-combustion engine crankshafts, for example with a thickness of 3" or more.

This invention is characterized by the combination of the following factors:

(1) A specific composition whereby the complete absence of graphite in the castings, satisfactory casting properties, and a remarkable aptitude to diffused graphitization, are obtained. The following component quantities (by weight) are suitable for carrying out this invention:

|    | Percent      |
|----|--------------|
| Ca | 2 to 3.0     |
| Cu | 0.1 to 3.0   |
| S  | 0.01 to 0.20 |
| Si | 1 to 2.5     |
| Mo | 0.05 to 0.50 |
| P  | 0.02 to 0.15 |
| Mn | 0.1 to 2.5   |
| Mg | 0.03 to 0.2  |
| Fe | Balance      |

Magnesium acts in this case as an element providing the white structure. This action is paradoxical since it constitutes the essential element of spherical graphitization in the fabrication of the so-called spheroidal cast-iron. Other whitening elements, other than magnesium, or an association of whitening elements, may be used for achieving the same results, if desired.

In addition, Ca, Te, Se, Sn, Bi, Sb, either separately or in combination, may be used as partial or entire substitutes for magnesium, their quantity being the reactive equivalent of the quantity of substituted magnesium.

In this procedure molybdenum acts as a promoter of martensitic hardening, but other elements characterized by the same property may be substituted therefor in a quantity providing the equivalent capacity of action. In the case considered herein the law of partial or total substitution which was discovered according to the present invention is represented by the equivalence table here-

2

after, wherein the part or parts by weight of the elements relate to one part by weight of molybdenum:

Mo=1, Ni=4, Cu=10  
Mn=4, W=2, V=0.3

Silicon acts in this case as a promoter of graphitization, the latter occurring during the thermal treatment. Its action may be completed by the addition of one of the following elements:

10 Titanium, with a maximum quantity of 0.5% (by weight), or

Zirconium, with a maximum quantity of 0.5% (by weight), or

15 Aluminum, with a maximum quantity of 0.20% (by weight).

(2) The casting is stripped well before it has cooled down completely, and in any case at a temperature above the temperature of eutectoid transformation, for example when the casting temperature ranges from 750 to 1,000° C., the casting is then placed immediately after its stripping in an oven at a temperature ranging from 740 to 850° C.

(3) When the temperature of the casting has been stabilized in the waiting oven, the casting is hardened by immersion either in oil at a temperature between room temperature and 200° C., or in a salt bath at a temperature differing slightly from the  $M_S$  point, that is, at from 150 to 250° C., the martensitic structure being obtained in this case either by direct hardening or by stepwise hardening, according to the temperature of the hardening medium.

(4) As a possible step, the casting is subjected to a cold treatment at a temperature ranging from  $-10^{\circ}$  C. and  $-195^{\circ}$  C. for the purpose of transforming the austenite likely to remain in the hardened castings into martensite.

(5) The casting is then given a germination treatment at an accurately defined temperature depending on the composition of the cast-iron, this temperature always ranging from 425 to 500° C., for a time period of from 1 to 48 hours. This treatment may be followed by cooling to room temperature.

(6) Finally the casting is subjected to graphitization which is carried out at a relatively high temperature for a sufficient time period, these two parameters being defined as a function of the composition, casting procedure and thickness of the parts. A reduction of from 850° C. for about 8 hours to 1,100° C. for about 15 minutes may be contemplated, according to circumstances, which is considerably faster than in the case of malleable cast-irons.

The specific novelty of the present invention lies in the definitely unforeseen effects due on the one hand to the action of the hardening of the non-cooled casting and on the other hand to the presence of hardening elements.

As a matter of fact, a systematic study carried out according to the Jominy test utilizing the end hardening test proved that the influence of the conventional martensitic hardening elements, when the casting temperature is used, the austenitization being effected from melting, was increased considerably in relation to that of the same elements obtained by re-heating the cold castings for austenitization at a conventional temperature of from 50 to 100° C. above the transformation point when heating the casting.

The influence of the following elements, which is figured out in additional martensitic hardened depth per percentage of each element, is shown in the next table setting forth on the one hand the results obtained with the hardening of a non-cooled casting, and on the other hand the results obtained for an austenitization by re-heat-

ing to 830° C. of the cooled casting, followed by a hardening step:

|               | Austenization by reheating to 830° C. of cooled casting, with subsequent hardening | Austenization of non-cooled casting |
|---------------|------------------------------------------------------------------------------------|-------------------------------------|
| With 1% of Mn | Millimeters                                                                        | Millimeters                         |
| With 1% of Cu | 6<br>1.4                                                                           | 16<br>6                             |
| With 1% of Mo | 7                                                                                  | 68                                  |

As a consequence of this discovery, high martensitic hardenability castings are obtainable by using moderate quantities of hardening elements.

A typical example of a practical embodiment of the method of the present invention is given hereafter:

Castings having a diameter of 60 millimeters and a length of 200 millimeters, cast in core sand moulds, and having the following composition:

C=2.58%; Si=1.34%; Mn=1.08%; Cu=2.0%; Mo=0.35%

S=0.009%; P=0.044%; Mg=0.29%; Fe=the balance, are stripped ten minutes after the completion of the casting step proper, and cooled for 5 minutes in a calm air atmosphere, before being placed in an oven at 780° C. for 5 minutes for stabilizing their temperature; then these castings are immersed and hardened in oil at 180° C. for 7 minutes and finally cooled in calm air. The hardened casting is white to the heart without any trace of graphite, and its micro-structure consists of martensite with 10 to 20% of austenite, without pearlite to the heart.

The casting is then heated for 4 hours at 450° C. for germination and subsequently heated for 8 hours at 950° C. for graphitization. After cooling, the casting shows a very homogeneous structure from the heart to the skin and its number of graphite grains is 3,000 per square millimeter.

The mechanical characteristics of this material are as follows:

Tensile strength----- 90 kilograms per square millimeter=(128,000 p.s.i.).  
Elastic limit----- 70 kg./sq. mm. (99,561 p.s.i.).  
Elongation----- 6%.  
Yield point----- 40 kg./sq. mm. (56,892 p.s.i.).

These characteristics cannot be obtained in cast products of this size (diameter=60 mm.) if they have not received a whitening agent such as magnesium or undergone a thermal treatment comprising the above-described steps such as the hardening from the casting temperature.

I claim:

A high strength malleable iron casting having a thickness greater than  $\frac{3}{4}$  in. and which is white and free from graphite as cast, containing in addition to iron 2 to 3% carbon, 1 to 2.5% silicon, 0.1 to 2.5% manganese, 0.1 to 3% copper, 0.01 to 0.20% sulphur, and 0.02 to 0.15% phosphorus, a metal of the group consisting of titanium, zirconium and aluminum, in the amount of up to 0.5% in the case of titanium, up to 0.5% in the case of zirconium, and up to 0.20% in the case of aluminum, a whitening metal consisting of at least one member of the group consisting of magnesium, calcium, tellurium, selenium, tin, bismuth, and antimony, the quantity of said whitening metal being the reactive equivalent of 0.03 to 0.20% magnesium, and a promoter metal consisting of at least one member of the group consisting of molybdenum, nickel, copper, manganese, tungsten and vanadium, the quantity of said promoter metal being the reactive equivalent of 0.05 to 0.5% of molybdenum, said reactive equivalent of 1 part by weight of molybdenum being by weight for each of the other promoter metals, 4 parts of nickel, 10 parts of copper, 4 parts of manganese, 2 parts of tungsten and 0.3 part of vanadium, said casting having a structure resulting from treatment by the steps which comprise stripping the white casting from the mold at a temperature above the eutectoid transformation temperature which ranges from 750 to 1,000° C., immediately introducing said casting into an oven, stabilizing the temperature of said casting in said oven within the range of 740 to 850° C., effecting after said stabilizing martensitic hardening by immersion in a liquid medium at a temperature up to 250° C., nucleation tempering at a predetermined temperature within the range 425 to 500° C. for a period of time from 1 to 48 hours, and graphitizing annealing at a temperature within the range 850 to 1,100° C. for a period of time from 15 minutes to 8 hours, said casting containing after said treatment a very large number of very fine, uniformly-distributed, rounded graphite modules.

#### References Cited in the file of this patent

#### UNITED STATES PATENTS

- 2,578,794 Gagnebin et al. ----- Dec. 18, 1951  
45 2,595,567 Crome ----- May 6, 1952  
2,895,860 Peras ----- July 21, 1959  
2,899,346 Peras ----- Aug. 11, 1959

#### FOREIGN PATENTS

- 50 513,106 Great Britain ----- Oct. 4, 1939  
601,755 Great Britain ----- May 12, 1948  
768,207 Great Britain ----- Feb. 13, 1957